

June 10, 1941.

2,245,421

A. VON FRANKENBERG UND LUDWIGSDORF ET AL

METHOD OF MAKING DEFORMED STEEL TUBES

Filed Nov. 25, 1938



Fig. 1.



Fig. 2.



Fig. 3.



Fig. 4.



Fig. 5.

Inventor's

Albrecht von Frankenberg und Ludwigsdorf  
and Heinrich Projahn,

By

*Frankenberg*

Attorney

## UNITED STATES PATENT OFFICE

2,245,421

## METHOD OF MAKING DEFORMED STEEL TUBES

Albrecht von Frankenberg und Ludwigsdorf and  
Heinrich Projahn, Gelsenkirchen, Germany,  
assignors to United States Pipe and Foundry  
Company, Burlington, N. J.

Application November 25, 1938, Serial No. 242,384  
In Germany December 13, 1937

1 Claim. (Cl. 29—156)

Socket pipes and similar hollow bodies made of steel and with enlargements or reductions in cross-sectional area or with thickened or recessed portions were hitherto produced almost without exception by first rolling a continuous smooth walled pipe by means of some rolling process, and then producing, for example, the sockets on the ends or any thickenings of the wall thickness by widening, upsetting or pressing.

When casting socket pipes and the like an entirely different process is employed in that the sockets or thickened portions of the pipes are cast directly in the corresponding casting process, as is known for example in the upright casting process and also in the centrifugal casting process for the production of cast-iron socket pipes and the like.

Although many suggestions have been made for producing steel pipes also by the centrifugal casting process, such great difficulties have been encountered in carrying out these suggestions in practice that up to the present there has been no real production of steel pipes, steel socket pipes or the like by the centrifugal casting process. Thus, for example it has been proposed to first centrifuge relatively thick-walled hollow blocks of steel and to then convert these centrifuged hollow blocks into their final shape by subsequently reducing their wall thickness along their entire length and over their entire cross-sectional area by rolling or drawing. Inaccuracies in the external diameter, in the wall thickness and defects such as flaws in the outer surface could be ignored, because the centrifuged intermediate products were subsequently subjected to a rolling or drawing process all over. This method of producing steel pipes is, however, relatively complicated and expensive.

Very recently it has been possible to produce by the centrifugal casting process satisfactory steel pipes complying with all requirements, true to measure and with faultless surfaces, by a special lining in the casting mould, which lining consists of loosely introduced granular substances which by correspondingly high circumferential speed are held together sufficiently tightly to resist washing away.

When centrifuging steel socket pipes are similar hollow bodies with different cross-sectional areas or different diameters at different points of their length, it is obvious to use correspondingly shaped centrifuging moulds, and to cast the sockets or the like directly on the steel pipes during the centrifugal casting process, as in

the known centrifugal casting process for cast-iron socket pipes.

It has, however, been found that owing to the relatively great shrinkage of the steel in solidifying (as compared with cast-iron) very fine cracks easily occur at the junctions between the pipe body and the pipe socket and even in the socket itself owing to the greater quantities of material at these points, which cracks may impair the appearance and the usefulness of the pipes.

To eliminate this possibility, it is proposed, according to the invention, to produce steel socket pipes and similar hollow bodies with enlargements or reductions in cross-sectional area or with thickened or recessed portions relatively short in axial directions, but, however, of uniform cross-section along relatively long sections of their length. This is realised by first producing by the centrifugal casting process the pipes or hollow bodies with substantially smooth continuous wall surfaces possessing the final cross-sectional dimension of their long part of uniform cross-section, whereupon only the socket-like widened, thickened or narrowed or similar portions necessary for the finished product are produced in known manner by mechanical deformation, such as widening, forging, upsetting, rolling or pressing, if necessary utilizing the heat remaining in the products from the casting operation.

At the same time these semi-finished products are centrifuged preferably in centrifugal moulds which have a centrifuged lining of loosely introduced granular substances, whose loose constituents, during the inflowing of the casting material, are held together sufficiently tightly by the correspondingly high circumferential speed to resist washing away by the inflowing jet of casting material.

According to the new process, it is possible for the first time to produce in a satisfactory manner steel socket pipes or similar hollow bodies having for example thickened or recessed portions or the like by the centrifugal casting process, a uniformly good quality of the product being ensured also on the socket portion or on the thickened or narrowed portion thereof owing to the subsequent formation only of the socket or thickened or narrowed portion or the like from the smooth pipe already centrifuged to measure.

As an example of an application of our invention, we would refer to the accompanying drawing in which

Figure 1 is a longitudinal section through the

center of a centrifugal pipe casting machine showing a housing, a rotatable mold mounted therein, a motor and gearing connections for rotating the mold, a trough supported from a movable carriage and inserted within the mold, means for feeding molten metal to the trough and means for tilting the trough, a mold lining preferably of loose granular material being also indicated as is also somewhat diagrammatically indicated the cast steel tube.

Figure 2 is a transverse section on line 2—2 of Fig. 1, through the mold and trough on an enlarged scale.

Figure 3 is a similar view to Fig. 2, showing the trough partially tilted and spilling molten metal into the mold.

Figure 4 is a perspective view of a length of pipe cast by the mechanism illustrated in Fig 1.

Figure 5 is a longitudinal section through the length of pipe shown in Fig. 4, and having a bell formed at one end thereof by expanding the end of the centrifugally cast pipe.

A is a housing, B a cylindrical mold mounted on said housing, B<sup>1</sup> an end ring in the form of a core located at one end of the mold and B<sup>2</sup> a metallic removable end ring located at the other end of the mold. C indicates a motor connected to rotate the mold through gearing as indicated at C<sup>1</sup>. D, a rotatable trough for delivering molten metal to the mold, supported as shown by a movable carriage D<sup>1</sup>, means for tipping the trough being diagrammatically indicated by the lever D<sup>2</sup>. E indicates means for supplying the rotatable trough with molten metal. f indicates the lining of the mold, F indicates the centrifugally cast steel tube or pipe which, as cast, is of uniform diameter and uniform wall thickness and F<sup>1</sup>, Fig. 5, indicates the same tube or pipe having one end expanded into the form of a bell or socket after the pipe is withdrawn from the mold.

The operation is, of course, obvious, the cen-

trifugal mold being in revolution at a satisfactory speed for the purpose, the molten steel is dumped into the rotating mold and centrifugally distributed over its surface to form a pipe or tube of uniform diameter and when the metal is set the pipe is withdrawn from the mold and such changes in its conformation as are desired are then brought about as shown and, by way of example, the only change noted is the expansion of one end of the pipe to form a bell or socket.

We claim:

A method of manufacturing steel tubes having a relatively long cylindrical section of substantially uniform wall thickness and a relatively short section differing therefrom in cross-sectional dimensions, which consists in providing a centrifugal mold with a lining formed of loosely introduced granular substances positioned and held in place against the washing effect of the molten steel introduced into the mold to form the casting by imparting to the mold during the pouring operation a rotary speed sufficient to hold the granular particles making up the lining in fixed position against the washing effect of the molten metal, centrifugally casting in the mold so lined a steel tube with substantially smooth, continuous wall surfaces and of substantially cylindrical shape throughout its length and of substantially uniform wall thickness and of mechanically deformable composition and structure, and then subjecting said relatively short section only of the cast tube while at suitable temperatures to a mechanical deforming operation to impart thereto cross-sectional dimensions differing from those of said relatively long cylindrical section, said relatively long cylindrical section being cast to substantially the final dimensions desired therefor.

ALBRECHT VON FRANKENBERG  
UND LUDWIGSDORF.  
HEINRICH PROJAHN.